

## UNITED STATES PATENT OFFICE

FRED SCHOLEFIELD, OF WALKDEN, ENGLAND, ASSIGNOR TO THE MANCHESTER OXIDE COMPANY LIMITED, OF MANCHESTER, ENGLAND

## OXIDATION PROCESS

No Drawing. Application filed June 27, 1928, Serial No. 288,815 and in Great Britain August 4, 1927.

This invention relates to improvements in oxidation processes in the dyeing or printing of textiles.

I have found that carbonylferrocyanides of the alkali metals, or alkaline earth metals have considerable catalytic or oxygen carrying properties, and can be employed to give catalytic or oxygen carrying effects in oxidation processes in the dyeing or printing of textiles.

In the dyeing and printing of aniline blacks on fabrics, by what is known as the "prussiate" process, an oxidizing material such as potassium chlorate together with sodium or potassium prussiate (ferrocyanide) has been mixed with the aniline salt.

The exact function of the prussiate is not known with certainty, but is usually considered to be of a catalytic or oxygen carrying nature. I have found however that if a carbonylferrocyanide is used instead of the prussiate, and, for this purpose we use sodium carbonylferrocyanide, although carbonylferrocyanides of the other alkalin metals, or alkaline earth metals may also be used, that advantages result, excellent aniline blacks being obtained on the fabric with greater certainty of control.

The following example in which the parts are given by weight illustrates the use of sodium carbonylferrocyanide in the dyeing of aniline black on fabrics, the sodium carbonylferrocyanide being employed instead of the usual prussiate.

The following solutions are prepared:—  
(a) A solution of 75 parts of aniline salt in 200 parts of water;  
(b) A solution of 35 parts of sodium chlorate in 400 parts of water; and  
(c) A solution of 30 to 40 parts of sodium carbonylferrocyanide in 250 parts of water.

When the solutions are quite cold they are mixed together. The cotton fabric to be dyed is padded through the mixed solutions, dried at a low temperature, steamed at a temperature of 90° C. and chromed in a 0.5% solution of bichromate of soda at a temperature of 50° C. The fabric is then well washed, soaped and dried.

In the chlorate discharge of such colors as

indigo and sulphur colors an oxidation effect is also obtained by means of an oxidizing agent and prussiate. As this process is usually carried out, the discharge portions of the fabric, especially in dark shades, often remain tinted instead of being pure white. I have found that by the addition of carbonylferrocyanides to the discharge paste instead of the prussiate, pure whites are readily obtained, a result not hitherto generally obtainable.

The following example in which the parts are given by weight illustrates the use of sodium carbonylferrocyanide in the chlorate discharge of indigo the sodium carbonylferrocyanide being employed in the place of the usual prussiate:—

200 parts British gum powder, 60 parts water, 550 parts chlorate of alumina (Sp. G. 42° Tw.) and 150 parts sodium chlorate are mixed together and boiled and after the mixture has been allowed to cool 30 to 40 parts sodium carbonylferrocyanide are added. The discharge paste thus formed is employed for the chlorate discharge of dark indigo dyed fabric being printed thereon in the usual way after which the fabric is dried and steamed for about 3 minutes in dry steam at a temperature of 100° C.

The cloth is then washed in water for five minutes at a temperature of between 60° to 80° C., passed through a caustic soda solution (4° Tw.) washed and dried.

I find that the use of carbonylferrocyanide to give catalytic or oxygen carrying effects in oxidation processes for textile purposes has an advantage over the use of prussiate, on the one hand, it is less active as an oxygen carrier in conjunction with chlorates at room temperatures. Consequently, aniline black padding liquors and printing pastes, containing carbonylferrocyanides are more stable at room temperatures, and may be kept for longer periods than the usual prussiate mixture without appreciable deterioration. Further, cloth padded with a solution in which ferrocyanide is replaced by carbonylferrocyanide is on and after drying, less liable to change in shade owing to premature oxidation of the aniline; and thus, cloths intended

for "discharge" effects, may be kept longer before printing the discharge paste, without risk of the production of poor whites. On the other hand it has greater activity at temperatures approximating to 100° C.

5 I have also found that when using carbonylferrocyanides there is less tendering of the fabric.

10 What I claim as my invention and desire to protect by Letters Patent is:—

15 1. A process for the production of aniline black on textile fibres in which a solution of an aniline salt, a solution of sodium chlorate and a solution of carbonylferrocyanide are mixed together and the fabric treated therewith.

20 2. A process for the production of aniline black on textile fibres in which a solution of an aniline salt, a solution of sodium chlorate and a solution of a carbonylferrocyanide of an alkali metal are mixed together and the fabric treated therewith.

25 3. A process for the production of aniline black on textile fibres in which a solution of an aniline salt, a solution of sodium chlorate and a solution of sodium carbonylferrocyanide are mixed together and the fabric treated therewith.

30 4. A process for dyeing of aniline black on textile fabrics in which a solution of an aniline salt, a solution of sodium chlorate and a solution of sodium carbonylferrocyanide are mixed together, the fabric impregnated with said mixture, dried at a low temperature and steamed.

35 5. A process for dyeing of aniline black on textile fabrics in which a solution of an aniline salt, a solution of sodium chlorate and a solution of sodium carbonylferrocyanide are mixed together, the fabric impregnated with said mixture, dried at a low temperature, steamed and chromed.

40 6. A process for dyeing of aniline black on textile fabrics in which a solution of an aniline salt, a solution of sodium chlorate and a solution of sodium carbonylferrocyanide are mixed together, the fabric impregnated with said mixture, dried at a low temperature, steamed, chromed, washed, soaped and dried.

45 In testimony whereof I have hereunto set my hand.

FRED SCHOLEFIELD.